

# UNITED STATES PATENT OFFICE.

ADRIEN BADIN, OF PARIS, FRANCE, ASSIGNOR TO SOCIÉTÉ GÉNÉRALE DES NITRURES, OF PARIS, FRANCE, A CORPORATION OF FRANCE.

## PROCESS OF MANUFACTURE OF ALUMINIUM NITRID.

1,143,482.

Specification of Letters Patent. Patented June 15, 1915.

No Drawing.

Application filed February 2, 1915. Serial No. 5,793.

*To all whom it may concern:*

Be it known that I, ADRIEN BADIN, a citizen of the Republic of France, and a resident of 12 Rue Roqu'épine, Paris, France, have invented a new and useful Process of Manufacture of Aluminium Nitrid, of which the following is a specification.

This invention relates to a process of manufacture of aluminium nitrid.

10 This process consists in this that there is caused to pass into a flame produced by the combustion of coal dust, an aluminous compound, for example bauxite, mixed with carbon, so as to be able to fix the nitrogen, 15 the quantity of air necessary for combustion being chosen in such a way that this combustion gives almost exclusively carbon monoxid. A combustion of this kind can be produced by causing to burn 100 kgs. of 20 coal by means of a quantity of atmospheric air which should be up to a maximum of 440 cubic meters.

To carry out the process, one adds to the 100 kgs. of coal dust above mentioned for 25 example a mixture finely pulverized of 30 kgs. of bauxite and of 12 kgs. of carbon. As the apparatus to be employed for this purpose, one may utilize any suitable coal dust furnace known in industrial applications.

30 The coal dust falls in the known manner from a hopper into a tube wherein it is carried along by air blown in. The coal dust is ignited at the end of the tube which delivers into a chamber preferably by means 35 of a flame produced by a suitable blowpipe, *e. g.* a heavy oil blowpipe, which it is advantageous to allow to burn continually in order to maintain, to render more active or to increase the combustion. Obviously there 40 may be also employed to this end a gas blow

pipe. (water gas, producer gas, etc.) or any blown flame. There is formed in the chamber, near the place where the pipe delivers, a flame of several meters, the length of which will vary according to the arrangement employed. The mixture of bauxite and of carbon blown in with the coal dust is carried along into the flame and a fixation of nitrogen takes place there. This effect is very surprising, for, according to data to 45 be found in books, the converting of coal, by its combustion, into carbon monoxid (CO) gives only a theoretical temperature of 1440° at which the fixation of nitrogen seems impossible, especially when there is present, as 50 is here the case, an important quantity of 55 oxid of carbon.

I claim:

1. A process of manufacture of aluminium nitrid, characterized by this that an aluminous material, mixed with carbon, is sent into a flame produced by the combustion of coal dust, the quantity of air for burning being chosen in such a way that the combustion gives almost exclusively carbon monoxid. 60

2. A process of manufacture of aluminium nitrid, characterized by this that bauxite, mixed with carbon, is sent into a flame produced by the combustion of coal dust, the 65 quantity of air for burning being chosen in such a way that the combination gives almost exclusively carbon monoxid. 70

In testimony whereof I have signed my name to this specification, in the presence of 75 two subscribing witnesses.

ADRIEN BADIN.

Witnesses:

CHARLES DONEY,  
DE WITT C. POOLE, Jr.

Copies of this patent may be obtained for five cents each, by addressing the "Commissioner of Patents, Washington, D. C."